

Feb. 7, 1933.

F. C. CRAWFORD

1,896,072

COPPER COOLED VALVE

Filed Feb. 13, 1931



Inventor

Frederick C. Crawford

By - Charles E. Kelly Attest.

## UNITED STATES PATENT OFFICE

FREDERICK C. CRAWFORD, OF CLEVELAND, OHIO, ASSIGNOR TO THOMPSON PRODUCTS, INCORPORATED, OF CLEVELAND, OHIO, A CORPORATION OF OHIO

## COPPER COOLED VALVE

Application filed February 13, 1931. Serial No. 515,567.

This invention relates to poppet valves for internal combustion engines and in particular to valves having a cooling medium therein.

5 The temperatures attained in the combustion chambers of automotive engines closely approximate the temperatures to which the metals used in the manufacture of valves are heated in such manufacture. The gases 10 which pass the exhaust valves maintain the exhaust passageway at a temperature of around 1600° F. for ordinary engine speed. These gases have a very destructive effect on 15 the valves causing corrosion and warping and producing a destructive change in the metal of the valve. Since these gases are directed against a portion of the valve which includes the upper portion of its stem and the lower portion of the head, it has been a 20 problem for valve manufacturers to devise a means of cooling this portion of the valve.

This cooling has been accomplished in several ways such as providing a shield about 25 this portion and also by filling the stem of the valve with a cooling medium which will draw the heat to a portion of the valve which may be cooled by outside means. The first 30 of these methods is objectionable because its effect depends upon the formation of a dead air space between the protecting shield and the valve. In this type of valve the heat being directed against the protecting shield will have a destructive action on the shield and will in time eliminate the dead air space. 35 The other method of cooling the valve, as heretofore practiced, while more permanent in nature, has been found not entirely satisfactory for the reason that it involves a considerable expense and careful planning or 40 else the cooling medium is not very effective.

According to the present invention, a simple and inexpensive means for cooling the portion of the valve against which the exhaust gases are directed is provided.

It is an object of this invention to provide a valve having a simple and effective cooling medium therein.

It is a further object of this invention to 50 produce a metallic cooled valve by a method

which is inexpensive, expedient and adapted for use in large scale production of valves.

It is a particular object of this invention to produce a valve of this type by a method which includes the welding of a cooling medium within the stem of the valve in such a manner as to produce a joint therebetween which has a very high rate of heat conductivity.

These and other objects of this invention 60 will appear from the following description and appended claims.

This invention (in a preferred form) is illustrated and described in this specification and accompanying drawing which forms a 65 part thereof.

On the drawing:

Figure 1 is a sectional view of a partially finished valve showing a copper rod inserted in a bore formed in the stem. 70

Figure 2 is a sectional view of an unfinished valve showing the copper rod welded therein.

Figure 3 is a sectional view of an unfinished valve showing a bore formed therein 75 by drilling a recess in the copper.

Figure 4 is a sectional view of an unfinished valve showing a result of a further step in forming the valve.

Figure 5 is a sectional view of a completed 80 valve.

As shown on the drawing:

In carrying out this invention, a member 1 of the general shape of a valve is formed in the usual manner of valve making as by 85 forging a blank or upsetting a rod. The metal blank in this stage of the operation is formed with a stem 2 and a head 3. A portion 4 of enlarged diameter is left at the end of the stem. 90

A bore or recess 5 is drilled through the end of the stem and extends throughout the length of the stem. The bore 5 is preferably cylindrical in shape. A copper rod 6 which is of sufficiently large diameter to snugly fill 95 the bore and of greater length, is inserted into the recess 5. The rod 6 may be of any metal having a very high rate of conductivity, but copper or a copper alloy is the most satisfactory.

The valve 1 is then placed on its head end into a furnace in which an atmosphere of hydrogen or other non-oxidizing, and preferably, reducing atmosphere, is maintained. 5 A small amount of a suitable flux 7 is applied to the copper insert adjacent the end of the valve. The furnace is then brought to a temperature slightly higher than the melting point of copper, about 2000° F. being the 10 preferable temperature. The copper is thereby caused to melt and settle down into the stem of the valve, entirely filling it. Due to the hydrogen atmosphere maintained in the furnace no oxidation can take place. 15 As a result of this operation the copper brazes itself to the steel and forms a perfect joint 8. The flux 7 flows down along the copper and the joint which is formed throughout the extent of the contacting steel 20 and copper surfaces, has no oxidized portions or air pockets. The result is a bond between the copper and the steel which has a rate of heat conductivity of approximately 97% of that of the steel alone, whereas ordinarily even a welded joint will offer a very 25 material resistance to the flow of heat.

After this operation the valve is removed from the furnace and the center of the copper is drilled out leaving a copper shell 9 30 permanently brazed or welded to the steel. The term "welded" is used here and in the claims to include any method wherein heat is used to effect a bond between the metal of the insert and of the wall of the stem. 35 The valve is again reheated and the thickened portion 4 of the stem worked down, as by swaging, to the diameter of the remaining portion of the stem. In this operation the metal of the enlarged portion 4 is 40 used to close the bore of the stem as shown at 10. The end of the copper shell 9 is drawn out as shown at 11 so as to form a solid closure for the stem.

The valve head is then worked into the 45 finished shape as shown at 12 and the stem end may be suitably threaded as shown at 13. A wearing surface 14, comprising a disc of metal, is preferably spot welded to the stem of the finished valve.

50 The valve produced by this method is very effective in conducting the heat from the portion of the valve in contact with the hot exhaust gases to other portions of the valve which may be cooled by external means. The 55 conductivity of the copper shell is approximately ten times that of the metals ordinarily used in the making of valves. The joint between the copper and the outer metal of the valve has a rate of heat conductivity 60 of about 97% of the rate of heat conductivity of the outer metal. A loose joint between copper and steel has a conductivity of about 40%.

65 It will thus be seen that this invention provides a self contained metal cooled valve

which is economical in its manufacture and efficient in use.

Many changes may be made in the design and proportion of parts, and I do not wish to be limited otherwise than is necessary by 70 the prior art and the scope of the appended claims.

I claim as my invention:

1. As a new article of manufacture, a hollow stem valve having a metal shell with- 75 in said hollow stem welded to the walls thereof.

2. As a new article of manufacture, a valve having a hollow stem and a metal shell with- 80 in said stem welded to the wall thereof with a non-oxidized bond between the shell and the wall of the valve stem.

3. A valve having a recess in the stem thereof, a copper shell within and completely filling said recess, said shell being welded to 85 the wall of said recess at all points to provide a non-oxidized bond therebetween.

In testimony whereof I have hereunto sub- 90 scribed my name at Cleveland, Cuyahoga County, Ohio.

FREDERICK C. CRAWFORD.

90

95

100

105

110

115

120

125

130